

[54] MEMBRANE FOR AN  
IN-VITRO-RESORPTION MODEL OF THE  
GASTROINTESTINAL TRACT[75] Inventor: **Herbert Stricker**, Ingelheim am  
Rhein, Germany[73] Assignee: **C. H. Bolhringer Sohn**, Ingelheim  
am Rhein, Germany[22] Filed: **July 27, 1971**[21] Appl. No.: **166,350****Related U.S. Application Data**[63] Continuation-in-part of Ser. No. 861,777, Sept. 29,  
1969, Pat. No. 3,612,283.[30] **Foreign Application Priority Data**

Sept. 27, 1968 Germany ..... P 17 98 340.3

[52] U.S. Cl. .... **210/490, 210/506**[51] Int. Cl. .... **B01d 39/14, B01d 31/00**[58] Field of Search. .... **210/23, 321, 490,  
210/491, 500, 506**[56] **References Cited**

## UNITED STATES PATENTS

3,612,283 10/1971 Stricker ..... 210/490

Primary Examiner—Frank A. Spear, Jr.

Attorney—Hammond &amp; Littell

[57] **ABSTRACT**

A porous membrane adapted for use as the filter element in an in-vitro-resorption model of the gastrointestinal tract, said membrane consisting essentially of solid porous carrier material, especially porous cellulose nitrate, impregnated with a liquid phase consisting of a mixture of (1) a higher fatty acid, such as caprylic acid, or dioctyl sodium sulfosuccinate and (2) a neutral lipid component, such as lauryl alcohol.

2 Claims, 2 Drawing Figures



PATENTED AUG 21 1973

3,753,501



FIG. 2



## MEMBRANE FOR AN IN-VITRO-RESORPTION MODEL OF THE GASTROINTESTINAL TRACT

This is a continuation-in-part of copending application Ser. No. 861,777, filed Sept. 29, 1969, now U.S. Pat. 3,612,283, issued Oct. 12, 1971.

### BACKGROUND OF THE INVENTION

The effectiveness of a drug in the system of the human body is, *inter alia*, a function of its concentration at the place of effective action and thus also a function of its ability to reach that place. Most of the perorally administered drugs must first overcome the barriers of the gastrointestinal tract, *i.e.*, they must be resorbed, before they can be transported by the blood to the place where they exert their therapeutic action.

Various *in-vivo* methods for following the passage of chemo-therapeutics from the gastrointestinal tract into the blood circulation system are known.

For instance, the decrease in the concentration of the chemo-therapeutic substance with passage of time in various parts of the gastrointestinal tract after peroral administration can be determined by analytical methods in the tied-off stomach, colon or small intestine of rats.

In humans, the change in concentration of various dissolved organic acids and bases in the stomach over a period of time can also be followed by means of an esophageal sound lowered into the stomach.

Likewise, in humans as well as animals, the blood level values at various times after peroral administration of drugs can be determined, from which rate of resorption can then be calculated.

Such *in-vivo* methods, however, require a substantial expenditure of work and money, and the results obtained therefrom are often subject to wide variations with respect to accuracy and reproduceability.

*In-vitro* methods employing artificial membranes, on the other hand, represent a valuable supplementation of the *in-vivo* determinations. Thus, by means of greater series tests and more accurate concentration determinations, the kinetics of diffusion can be very accurately ascertained, so that the effects of the interchange action between the active ingredients among themselves or with the pharmaceutical excipients can already be evaluated and taken into consideration in determining the most favorable make-up of the pharmaceutical dosage unit compositions. Moreover, by employing *in-vitro* methods, the number of *in-vivo* tests can be significantly reduced.

### THE PRIOR ART

Filter membranes for various purposes have already been described in the literature. For instance, porous membranes made of cellulose esters and impregnated with olive oil or linoleic acid have been described by G. Levy and E. J. Mroszezak in *J. Pharm.Sci.* 57(2), 235-239 (1968).

However, it was found that, while these olive oil-impregnated filter membranes are "pH-impermeable," they also do not permit the passage of substances of an acid character if they are present in weakly acid to neutral solution. Therefore, the olive oil-impregnated membranes are not well suited for *in-vitro* resorption tests, especially if the apparatus is to simulate resorption in the small intestine.

On the other hand, linoleic acid-impregnated membranes proved to be insufficiently permeable with re-

spect to hydrogen or hydroxyl ions, so that they could not be used for diffusion measurements between solutions having a different pH-value.

### OBJECTS OF THE INVENTION

The present invention has as its principal object to provide a membrane for use in an *in-vitro* resorption test apparatus, which is capable of maintaining the pH-gradient between two aqueous solutions substantially constant over a period of time of about 50 hours and exhibits a specific permeability for acid, basic and amphoteric drug molecules.

Another object of the instant invention is to provide a porous membrane for use in an *in-vitro* resorption test apparatus, which duplicates as closely as possible the drug diffusion rates under physiological conditions known from *in-vivo* tests.

Other objects and advantages of the invention will become apparent as the description thereof proceeds.

### THE INVENTION

The above objects are achieved in accordance with the present invention by impregnating a solid porous carrier material with a liquid lipoid phase.

The porous carrier material may be a commercial membrane filter material made of a cellulose ester. The diameter of the pores must be sufficiently small so that the pores, due to their capillary activity, remain closed by means of the liquid impregnation component; otherwise, the liquid impregnation phase could be dissolved out and the membrane would become useless. Therefore, the diameter of the pores should be from 50 to 1,000 mu, preferably 100 mu. Examples of suitable membrane filter material are the commercially available products Millipore VC and Sartorius SM 11309.

The liquid lipoid phase must resemble, with respect to its physical properties, such as its relative solution capacity for acid, basic and amphoteric drugs, and its distribution, as closely as possible to its natural counterpart, *i.e.* the stomach and intestinal walls, so that the relative resorption rates of various drugs can be accurately simulated in the *in-vitro* apparatus.

I have found that these requirements are met by a mixture consisting of (1) a higher fatty acid, preferably caprylic acid, or dioctyl sodium sulfosuccinate, and (2) a neutral lipoid component, such as a higher fatty alcohol of 12 or more carbon atoms, preferably lauryl alcohol. The mixture of these two components must be liquid at the test temperature of 37°C.

A membrane according to the present invention is prepared by immersing the porous filter material into said liquid mixture, removing the impregnated porous material from the liquid mixture and allowing excess liquid mixture to drip off, and blotting the impregnated porous membrane between filter paper until its weight is constant. A preferred embodiment of the membrane is obtained by using as the liquid impregnating component a mixture of 80 parts by volume caprylic acid and 20 parts by volume lauryl alcohol, or a mixture of 97 parts by volume lauryl alcohol and three parts by volume dioctyl sodium succinate.

In contrast to known membranes of this type, membranes in accordance with the present invention have the advantage that they are capable of maintaining the pH-gradient between two aqueous solutions substantially constant ( $\pm$  about 0.3 pH-units) over a period of about 50 hours and exhibit a specific permeability for

acid, basic and amphoteric drug molecules. The diffusion rates under physiological conditions correspond substantially to the values known from in-vivo tests.

The combination of a higher fatty acid or dioctyl sodium sulfosuccinate and a neutral lipid component with a cellulose ester filter membrane as a carrier material proved to be a system which meets the requirements surprisingly well. The effect of the fatty acid or sulfosuccinate component is that, corresponding to its  $pK_a$ -value and the pH of the adjacent solution, it is partly present as an anion and acts as a proton-acceptor or -donor with respect to the dissociated organic acids or bases. The drugs are thereby transformed at the membrane surface into the undissociated form and are thus capable of migrating through the liquid phase of the membrane, whereas the hydrogen and hydroxyl ions can pass through only very slowly because of the solubility conditions.

The annexed drawings show schematically the type of in-vitro diffusion apparatus wherein a membrane according to the present invention can be used.

FIG. 1 is a schematic representation of an apparatus which consists essentially of two chambers 1 and 1a (volume of each 100 ml) which are separated by a membrane 2 according to the present invention (effective surface  $12.5 \text{ cm}^2$ ). Each of the chambers is provided with a thermostatically controlled exterior heating jacket 3 to maintain the contents at  $37 \pm 0.5^\circ\text{C}$ . Two pipettes 4 and 5 extend into each of the chambers 1 and 1a, and a dropping funnel (not shown) is connected to the exterior end of each pipette. The flow of liquid through each pair of pipettes is controlled by a double stopcock 6. Pipettes 5 terminate substantially at the point where they enter chambers 1 and 1a, respectively, whereas pipettes 4 extend into the respective chambers to a point close to the surface of membrane 2. One of the two chambers 1 and 1a is filled with a physiological solution having a pH of 7.5, which corresponds to that of blood plasma; the other chamber is filled with a physiological solution whose pH is adjusted to between 1.2 and 7.0, depending upon the section of the gastrointestinal tract which it is intended to duplicate. The dropping funnel connected to each of the short pipettes 5 is filled with buffer solution to maintain the pH in each chamber at the desired level. A metal disc 7 having a central aperture is slidably mounted on each pipette 4. The entire apparatus is mounted so that it oscillates 36 times per minute through an angle of  $170^\circ$  about a transverse axis 8 which coincides with the center of the plane formed by membrane 2, the oscillating motion being provided by a motor (not shown). By virtue of this oscillating motion the metal discs 7 slide along pipettes 4 and thereby stir the solution in each chamber. In order to withdraw a sample of the solution in chamber 1 or 1a, the respective double stopcock 6 is opened, whereby the descending buffer solution in pipette 5 forces some solution from the chamber upward through pipette 4 into the dropping funnel connected thereto, wherefrom it can be withdrawn for analysis. At the same time the solution in the chamber is replenished with fresh buffer solution. The function of membrane 2 is to maintain the pH-gradient between the solutions in chambers 1 and 1a, and also to permit differential passage of various drugs, i.e., organic acids and bases of different types. The drug whose diffusion rate is to be tested is introduced into the solution which duplicates the particular section of the intestinal tract.

FIG. 2 is a schematic representation of another diffusion apparatus which comprises a diffusion vessel 9 consisting of two chambers 10 and 10a separated by a membrane 11 according to the present invention. The test solutions are cycled by means of pump 12 from storage vessels 13 and 13a into chambers 10 and 10a, respectively, and then back into the storage vessels. The cycling rate depends on the dimensions of the apparatus; for example, if the membrane surface is about  $12 \text{ cm}^2$  and the volume of chambers 10 and 10a is about 2 to 5 ml each, the cycling rate is advantageously about 2 to 10 ml/min. In addition, the solutions in storage vessels 13 and 13a are continuously stirred by means of a magnetic stirrer 14 in order to avoid concentration gradients. Thermostatically controlled heating jackets 15 maintain a constant temperature of  $37^\circ\text{C}$ . Stopcocks 16 permit withdrawal of samples of the solutions for analysis.

The following examples further illustrate the present invention and will enable others skilled in the art to understand it more completely.

#### EXAMPLE 1

Using a diffusion test apparatus such as the one shown in FIG. 1 of the drawings, the resorption rate of various acid and basic drugs from the stomach was tested.

The membrane was a porous sheet of cellulose nitrate, pore size  $100 \pm 8 \text{ \mu m}$  (Millipore VC or Sartorius SM 11309), impregnated with a liquid mixture consisting of 50 parts by volume of caprylic acid and 50 parts by volume of lauryl alcohol.

One diffusion chamber was filled with a solution of the drug compound in 100 ml of a buffer solution having a pH of 1.2, i.e., the pH prevailing in the stomach, prepared from 24 gm of 1 N HCl, 0.5 gm of glycocoll, 0.35 gm of NaCl and enough  $\text{H}_2\text{O}$  to make 1,000 ml.

The other diffusion chamber was filled with 100 ml of a buffer solution having a pH of 7.5, prepared from 20.5 gm of  $\text{Na}_2\text{HPO}_4$ , 2.7 gm of  $\text{KH}_2\text{PO}_4$  and enough  $\text{H}_2\text{O}$  to make 1,000 ml.

The apparatus was oscillated as described above in connection with FIG. 1 of the drawings, and samples of the solution in each chamber were withdrawn periodically, while at the same time replenishing the buffer solution from the dropping funnels.

The following table shows the results obtained in comparison to known in-vivo resorption rates, all values being based on the resorption rate of aspirin = 1.00

T A B L E I

| Compound             | Initial Resorption Rate, based on rate of acetylsalicylic acid = 1.00 |          |
|----------------------|-----------------------------------------------------------------------|----------|
|                      | in-vivo*                                                              | in-vitro |
| Acetylsalicylic acid | 1.00                                                                  | 1.00     |
| Salicylic acid       | 2.3                                                                   | 2.3      |
| Benzoic acid         | 2.0                                                                   | 2.2      |
| Phenol Red           | 0.05                                                                  | 0.1      |
| Aminopyrine          | 0.05                                                                  | 0.0      |
| Quinine              | 0.00                                                                  | 0.0      |
| Ephedrine            | 0.00                                                                  | 0.0      |

\* L. S. Schanker et al., J. Pharm. exp. Therap. 120, 528 (1958).

#### EXAMPLE 2

The test procedure and apparatus were the same as in Example 1, except that the membrane was impregnated with a liquid mixture consisting of 20 parts by

volume of lauryl alcohol and 80 parts by volume of caprylic acid, and the buffer solution having the drug compound dissolved therein had a pH of 6.0 to simulate conditions in the small intestine; the buffer solution was prepared from 1.5 gm of  $\text{Na}_2\text{HPO}_4$ , 80 gm of  $\text{KH}_2\text{PO}_4$  and enough water to make 1,000 ml.

The following results were obtained:

T A B L E II

| Compound             | Initial Resorption Rate, based on rate of acetylsalicylic acid = 1.00 |          |
|----------------------|-----------------------------------------------------------------------|----------|
|                      | in-vivo*                                                              | in-vitro |
| Acetylsalicylic acid | 1.00                                                                  | 1.00     |
| Benzoinic acid       | 2.9                                                                   | 2.7      |
| Barbital             | 1.5                                                                   | 1.4      |
| Phenol Red           | 0.2                                                                   | 0.2      |
| Aminopyrine          | 1.9                                                                   | 2.0      |
| Ephedrine            | 0.3                                                                   | 0.2      |
| Theophylline         | 1.4                                                                   | 1.1      |
| Antipyrine           | 1.7                                                                   | 1.3      |

\* L. S. Schanker et al., J. Pharm. exp. Therap. 120, 528 (1958).

## EXAMPLE 3

The test procedure and apparatus were the same as in Example 1, except that the membrane was impregnated with a liquid mixture consisting of three parts by volume of diocetyl sodium sulfosuccinate and 97 parts by volume of lauryl alcohol.

The following results were obtained:

T A B L E III

| Compound             | Initial Resorption Rate, based on rate of acetylsalicylic acid = 1.00 |          |
|----------------------|-----------------------------------------------------------------------|----------|
|                      | in-vivo*                                                              | in-vitro |
| Acetylsalicylic acid | 1.00                                                                  | 1.00     |
| Benzoinic acid       | 2.9                                                                   | 2.7      |
| Barbital             | 1.5                                                                   | 1.4      |
| Phenol Red           | 0.2                                                                   | 0.2      |
| Aminopyrine          | 1.9                                                                   | 2.0      |
| Ephedrine            | 0.3                                                                   | 0.2      |
| Theophylline         | 1.4                                                                   | 1.1      |
| Antipyrine           | 1.7                                                                   | 1.3      |

\* L. S. Schanker et al., J. Pharm. exp. Therap. 120, 528 (1958).

|                     | in-vivo* | in-vitro |
|---------------------|----------|----------|
| Acetylcyclonic acid | 1.00     | 1.00     |
| Salicylic acid      | 2.30     | 2.10     |
| Benzoic acid        | 2.00     | 2.10     |
| Phenol Red          | 0.05     | 0.05     |
| Aminopyrine         | 0.05     | 0.02     |
| Quinine             | 0.00     | 0.00     |
| Ephedrine           | 0.00     | 0.00     |

\* L. S. Schanker et al., J. Pharm. exp. Therap. 120, 528 (1958).

The results of these examples clearly show that, with the aid of an in-vitro apparatus comprising a membrane according to the present invention it is possible to duplicate very closely the in-vivo resorption conditions of the gastrointestinal tract.

15 While the present invention has been illustrated with the aid of certain specific embodiments thereof, it will be readily apparent to others skilled in the art that the invention is not limited to these particular embodiments, and that various changes and modifications may be made without departing from the spirit of the invention or the scope of the appended claims.

I claim:

1. A membrane for an in-vitro resorption model of the gastrointestinal tract, said membrane consisting of a porous cellulose ester filter membrane material having a pore size of 0.05 to 1.0  $\mu$  impregnated with a mixture consisting of diocetyl sodium sulfo-succinate and lauryl alcohol, said mixture being liquid at 37°C.

2. A membrane according to claim 1, wherein said liquid mixture consists of 3 percent by volume of diocetyl sodium succinate and 97 percent by volume of lauryl alcohol.

\* \* \* \* \*